

## UNITED STATES PATENT OFFICE

LUDWIG KERN AND FERNANDO C. KERN, OF WEBSTER GROVES, MISSOURI

BINDER MATERIAL FOR COAL, COKE, AND THE LIKE, AND THE MANUFACTURE  
THEREOF

No Drawing.

Application filed June 18, 1930. Serial No. 462,128.

This invention relates to binder materials for pulverized coal, coke and the like, and with regard to certain more specific features, to non-smoke producing binder materials.

5 Among the several objects of the invention may be noted the provision of a binder material of non-smoke producing characteristics which is made from readily obtainable material normally discarded at coal mines; 10 a binder material which is readily adaptable to varieties of coal with beneficial results; a binder material which, when utilized with coal, coke and the like, produces a bound product of high compressive strength, un- 15 usual hardness and wear-resisting qualities; the production as a by-product of a highly useful decolorizing and deodorizing pulverized filtering material; and the provision of 20 a process for manufacturing a binder material of the class described which is easily and economically carried through, and which requires a minimum of expensive treating materials and the like. Other objects will 25 be in part obvious and in part pointed out hereinafter.

The invention accordingly comprises the elements and combinations of elements, steps and sequence of steps and features of synthesis which will be exemplified in the description hereinafter and the scope of the application of which will be indicated in the following claims.

Certain types of coals, ordinarily termed "non-coking" coals, destructively distill to 30 form unsatisfactory coke of low compressive strength, low wear-resisting qualities, and the like. It has been proposed to use binder materials, such as liquefied asphalt, pitch, tar, oils, naphthalene, or resins, in order to 35 bind the coal into satisfactory lumps for coking. In general these binder materials are only partially satisfactory, and do not lead to a hard coke. Additional disadvantages include the predominant smoke-producing characteristics of such binder materials, which render the product unfit for 45 commercial utilization in large cities and the like.

The present invention provides a binder material for non-coking coals which binds 50 said coals to effect a hard, firm coke as here-

inbefore described, and which is not smoke-producing in its characteristics.

Ordinary bituminous coal exists in geologic strata which are imbedded in and interspersed with clays, shales, and other earthy 55 materials, generally termed "coal shales" or "gangue material". This gangue material in general comprises hydrates, oxides, carbonates, and silicates of aluminum, calcium, magnesium, sodium and iron. Impurities 60 are variable; contents of silicia, sand, pyrites, and organic or carbonaceous materials are not uncommon.

This gangue material, not necessarily cleaned or freed of its carbonaceous adher- 65 ents, is finely ground and freed so far as possible from its impurities. The impurities may be removed by such means as air or liquid floatations, washers, and the like. The cleaned material is then boiled in a closed container 70 with hydrochloric acid, after which it is allowed to settle, and the supernatant liquid decanted or otherwise removed therefrom. The solid residue is washed and passed 75 through a filter press.

The supernatant liquid comprises a concentrated, viscous solution of the chlorides of the metals forming the gangue material. In general, the principal constituents are aluminum, calcium, magnesium, sodium, and iron 80 chlorides, and free hydrochloric acid. This liquid constitutes a valuable binder and plasticizer material for comminuted coal, whereby it can be formed into briquettes and effectively coked. The solution presumably functions as a binder material by reacting with and plasticizing the ash-forming constituents of the coal. It is to be understood that the supernatant liquid may be concentrated 85 or diluted, as individual cases may require. 90

The solid material left behind after the supernatant liquid has been decanted is preferably washed until only faintly acid, passed through a filter press, and dried and powdered. The powder in general comprises hydrochloric acid-insoluble materials, together with residues of unattacked acid-soluble materials, and carbonaceous matter. The powder is a valuable decolorizing and deodorizing agent to oils, fats, waxes and the like, and a 95

filter material for natural and synthetic dyes, especially of an alkaline nature.

It is to be understood that, if desired, the acid solution need not be decanted, but may be used as a binder material with the undissolved residue still therein.

A specific example of the invention is as follows:

Illinois coal mine clay is ground to a fineness of from 100 to 200 mesh, and treated in a clay washer to remove silica, sand, pyrites and gob. The washed clay is then mixed with from 50 to 100 per cent. by weight of aqueous hydrochloric acid of gravity 17° Bé. The mixture is boiled at about 100° C. for two hours or more, preferably with constant agitation. Water and/or more acid is added from time to time to keep up the proper volume. After the boiling is completed, the mixture is allowed to settle, and the supernatant solution drawn off or decanted. This solution is preferably then diluted to a gravity of the order of 4° to 6° Bé, in which condition it is used for plasticizing comminuted coal. The solid matter left after the decantation comprises about 70 per cent. silica, 4 per cent. iron oxide, 6 per cent. alumina, and the remainder carbonaceous materials and impurities. It is washed until the wash water shows only a slight acid reaction on litmus paper, then filtered and dried at temperatures not higher than the order of 85° C., and pulverized.

In view of the foregoing, it will be seen that the several objects of the invention are achieved and other advantageous results attained.

As many changes could be made in carrying out the above objects without departing from the scope of the invention, it is intended that all matter contained in the above description shall be interpreted as illustrative and not in a limiting sense.

We claim:

1. A binder material for pulverized coal and the like comprising an acid solution of coal gangue containing an excess of acid.

2. A binder material for pulverized coal and the like comprising a hydrochloric acid solution of coal gangue containing an excess of hydrochloric acid.

3. A binder material for pulverized coal and the like comprising a solution of the chlorides of metals present in coal gangue containing free hydrochloric acid.

4. A binder material for pulverized coal and the like comprising a hydrochloric acid solution of earthy materials containing free hydrochloric acid.

5. The process of manufacturing a binder material for pulverized coal and the like which comprises comminuting the gangue material ordinarily naturally associated with said coal, treating the pulverized gangue with hydrochloric acid whereby various con-

stituents of said gangue are dissolved, and removing said acid with the substances dissolved therein from the undissolved gangue.

6. The process of manufacturing a binder material for pulverized coal and the like which comprises comminuting the gangue material ordinarily naturally associated with said coal, boiling the pulverized gangue with hydrochloric acid whereby various constituents of said gangue are dissolved, and removing said acid with the substances dissolved therein from the undissolved gangue.

7. The process of manufacturing a binder material for pulverized coal and the like which comprises comminuting coal gangue to a fineness of the order of 100 mesh, boiling the comminuted gangue with from 50 to 100 per cent. of its weight of hydrochloric acid, whereby portions of said gangue are dissolved in said hydrochloric acid and removing said hydrochloric acid solution from the undissolved portion of said gangue.

8. The filter material which comprises comminuted coal gangue from which a substantial portion of the metallic constituents have been dissolved with hydrochloric acid.

9. The filter material which comprises comminuted coal gangue which has been treated with hydrochloric acid for the removal of a substantial portion of the metallic constituents.

10. The filter material which comprises a comminuted mixture of approximately 70% silica, 4% iron oxide, 6% alumina, and the remainder carbonaceous material.

In testimony whereof, we have signed our names to this specification this 13th day of June, 1930.

LUDWIG KERN.  
FERNANDO C. KERN.